

# United States Patent [19]

Goodfellow

[11] Patent Number: **4,607,515**

[45] Date of Patent: **Aug. 26, 1986**

[54] **KINETIC ENERGY PENETRATOR**

[75] Inventor: **Glenn B. Goodfellow, Franklin Lake, N.J.**

[73] Assignee: **UTI Corporation, Collegeville, Pa.**

[21] Appl. No.: **562,305**

[22] Filed: **Dec. 16, 1983**

**Related U.S. Application Data**

[63] Continuation-in-part of Ser. No. 451,136, Dec. 20, 1982, Pat. No. 4,462,238.

[51] Int. Cl.<sup>4</sup> ..... **B21D 22/00**

[52] U.S. Cl. ..... **72/358; 72/453.08; 72/354; 219/119**

[58] Field of Search ..... **72/352, 358, 359, 354, 72/360, 438, 453.08; 219/159.2, 119**

[56] **References Cited**

**U.S. PATENT DOCUMENTS**

2,169,113 8/1939 Sheppard ..... 72/453.08

|           |         |                        |          |
|-----------|---------|------------------------|----------|
| 3,167,859 | 2/1965  | Bailey .....           | 72/352   |
| 3,209,453 | 10/1965 | Bertoglio et al. ..... | 72/354   |
| 3,832,763 | 9/1974  | Schober .....          | 29/159.2 |
| 4,045,644 | 8/1977  | Shafer et al. .....    | 219/119  |

**OTHER PUBLICATIONS**

Brochure of Rheinmetall Wehrtechnik

Primary Examiner—W. D. Bray  
Attorney, Agent, or Firm—Seidel, Gonda, Goldhammer & Abbott

[57] **ABSTRACT**

A penetrator is made in accordance with a method for increasing strength and/or hardness of a metal specimen. Compressive force is applied to the specimen slowly so that the yield strength of the specimen progressively increases and the specimen exhibits squirming instability as its diameter increases. The penetrator is adapted to be fired from a smooth bore weapon.

**12 Claims, 16 Drawing Figures**





FIG. 2



FIG. 7



FIG. 12



FIG. 13



FIG. 14



FIG. 16



FIG. 15



## KINETIC ENERGY PENETRATOR

## RELATED CASES

This application is a CIP of application No. 451,136 filed Dec. 20, 1982 and entitled Method For Controlling Properties Of Metals And Alloys, now U.S. Pat. No. 4,462,238.

## BACKGROUND OF THE INVENTION

It is old and well known in the art of metal working to cold work metals and alloys. It is known from U.S. Pat. No. 3,209,453 to shape a blank in a die prior to finish machining. It is known from U.S. Pat. No. 4,045,644 to apply axial pressure on a sintered electrode blank to pressure flow the blank radially to reorientate the grain structure.

It would be highly desirable if one could control mechanical properties of metals in a predictable manner so as to attain, for example, a metal penetrator having predetermined variable strength along its entire length or along only a portion of its length. The present invention is directed to attaining that goal.

## SUMMARY OF THE INVENTION

The present invention is directed to a kinetic energy penetrator made in accordance with a method for increasing strength and/or controlling mechanical properties of metals and alloys in a predictable manner as disclosed in said patent applications. A specimen is produced with a preshape and dimensions determined on the basis of the desired strength or mechanical properties with the specimen length being substantially greater than the transverse dimensions. The preshaped specimen is introduced into a confined chamber which defines the desired final shape. At least a portion of the specimen is spaced from the periphery of the walls defining the chamber with the relative dimensions of the spacing being governed by the amount of cold work needed to achieve desired strength or mechanical properties in that portion of the specimen.

One face of the specimen is engaged with a moveable wall of the chamber. The moveable wall of the chamber applies a continuous compressive force with a sufficient magnitude so as to force the preshaped specimen to deform and fill the chamber at the end of the compressive stroke while simultaneously decreasing length and maintaining the volume of the specimen constant. The compressive force is applied at a rate so that the yield strength of the preshaped specimen progressively increases. At the same time, the compressive force progressively increases as the yield strength increases until the entire circumference of the specimen contacts the walls of the chamber and attains said desired final shape at the end of the compressive stroke. The thusly produced specimen is used to produce a penetrator.

It is an object of the present invention to provide a kinetic energy penetrator.

It is another object of the present invention to provide a penetrator having predictably controlled mechanical properties such as strength or hardness along the length thereof.

Other objects and advantages will appear hereinafter.

## DESCRIPTION OF THE DRAWINGS

FIG. 1 is a sectional view of a closed die containing a specimen.

FIG. 2 is an elevation view of the specimen in FIG. 1 after it has been shaped.

FIG. 3 is a sectional view of a closed die containing another specimen.

FIG. 4 is an elevation view of the specimen in FIG. 3 after it has been shaped.

FIG. 5 is a sectional view of a closed die containing another specimen.

FIG. 6 is an elevation view of the specimen in FIG. 5 after it has been shaped.

FIG. 7 is a sectional view of a closed die containing another specimen.

FIG. 8 is an elevation view of the specimen in FIG. 7 after it has been shaped.

FIG. 9 is a sectional view of a closed die containing another specimen.

FIG. 10 is an elevation view of the specimen in FIG. 9 after it has been shaped.

FIG. 11 is a perspective view of a specimen showing the spiral pattern resulting from squirming instability.

FIG. 12 is a graph of elongation versus percent increase in area by cold working a 91% tungsten alloy.

FIG. 13 is a graph of ultimate tensile strength versus percent increase of cross-sectional area by cold working a 91% tungsten alloy.

FIG. 14 is a graph of hardness versus percent increase in cross-sectional area by cold working a 91% tungsten alloy.

FIG. 15 is a diagrammatic illustration of a penetrator being fired from a smooth barrel weapon.

FIG. 16 is an elevation view of the penetrator with a sabot assembled thereto.

## DETAILED DESCRIPTION

Referring to the drawing in detail, wherein like numerals indicate like elements, there is shown in FIG. 1 a portion of a press 10 having a confined chamber 12 defined at its ends by walls 14 and 16. At least one of the walls, such as wall 16 is moveable toward and away from the wall 14. Within the chamber 12, there is provided a specimen 18 of a metal to be cold worked.

The specimen 18 is preformed with a cylindrical shape. The chamber 12 defines the desired peripheral final shape for the specimen and likewise in this embodiment is a cylinder. Wall 16 engages one end face of the specimen 18 and applies a continuous compressive force with a sufficient magnitude to force the preshaped specimen 18 to deform and fill the chamber 12 at the end of the compressive stroke. The specimen 18 simultaneously decreases length while maintaining its volume so as to have a final shape as shown in FIG. 2 and designated 18'. The compressive forces of wall 16 are applied sufficiently slowly so that the yield strength of the specimen 18 progressively increases. This in turn requires the compressive forces to progressively increase in magnitude as the yield strength increases until the entire circumference of the specimen 18 contacts the walls of chamber 12 and attains the desired final shape at the end of the compressive stroke as shown in FIG. 2.

In virtually every engineering design problem encountered in real life situations, engineers and scientists strive for designs that preclude loading of columns or columnar type structures to levels where buckling can occur. Such column buckling has been well-known for 200 years.

Mathematical criteria for column buckling was first developed by L. Euler in 1744, and the governing equation has since been known as the Euler equation. It

states simply that a column must attain a certain length before it can be bent by its own or an applied weight.

The Euler formula has withstood the test of time. Originally it was stated as (1)

$$FL^2 > 4\pi^2 B,$$

where

F=load in pounds (lbs.)

L=length in inches

B=Flexural rigidity=EI(Lb-in<sup>2</sup>), where

E=Youngs Modulus of elasticity (Lb/in<sup>2</sup>)

I=Moment of inertia about the axis of bending (in<sup>4</sup>).

(1) A. E. H. Love, Mathematical Theory of Elasticity, Dover Publication 1974.

In its present day form, the equation (2) is given as

$$W_{CR} = K_C \frac{EI}{L^2}$$

where

$W_{CR}$ =Critical Load beyond which buckling will occur, and

$K_C$ =is a constant which depend upon the manner of support and loading.

In fact, the value of  $K_C$  for clamped or supported end conditions with axial load is given (2) as 39.48 which is exactly equal to  $4\pi^2$ , so that

$$W_{CR} = 4\pi^2 \frac{EI}{L^2}$$

is exactly the Euler equation.

(2) Alexander Blake, Practical Stress Analysis in Engineering Design, Marcel Dekker, Inc. 1982.

It is a fact emphasized in the literature that the critical buckling load  $W_{CR}$  is proportional to the Modulus of Elasticity E, section moment of inertia I, and inversely proportional to column length squared  $1/L^2$ , and is independent of yield strength of the material. It is further emphasized that critical buckling occurs at stress below uniaxial yield stress values.

I uniquely found that the amount of deformation force necessary to achieve the desired final geometry, and thus mechanical properties, can be achieved by exploiting those elements of column buckling which Engineering text books define as the forbidden zones. For example, tungsten base heavy metal alloy specimen with initial diameter of 0.32 inches, was placed in the press die having a diameter of 0.38 inches and compressive force applied axially. After compressing approximately 25% of the total deformation, it was found that deformation was not uniform compression. Rather, deformation occurred by apparent buckling until the die wall restraint was encountered after which the specimen continued to deform in a spiral-like fashion with quite uniform pitch from end to end. See FIG. 11. Final deformation occurred by compressive stress. For ease of reference, I define this spiral deformation cycle as squirming instability followed by compression until final geometry is achieved.

In a typical example, specimen 18 was made from a 94% tungsten base alloy with a length of 5.49 inches and a diameter of 0.345 inches. The specimen 18' had a length of 4.50 inches and a diameter of 0.381 inches. Hardness was very uniform along its entire length and varied between 39 and 40 R<sub>c</sub>.

In FIG. 3, there is illustrated a different specimen 20 in the chamber 12. Specimen 20 was smaller in diameter than specimen 18 and formed the specimen 20' after

compression and cold working. The effect on hardness was substantially the same as that attained in connection with FIGS. 1 and 2. However, as the percentage of cold working increased, the hardness likewise increased. See

5 FIG. 14.

In FIG. 5 there is shown a similar specimen 24 in the chamber 12. Specimen 24 is in the form of a truncated cone made from 94% tungsten alloy. After compression, the resultant specimen 24' is a cylinder but its 10 hardness progressively increases in a direction from its upper end to its lower end in FIG. 6 where the R<sub>A</sub> readings at A, B and C were 66, 69 and 72. The tensile strength at A was 135,000 psi with 25% elongation and at C was 200,000 psi with 2% elongation.

15 In FIG. 7, the press 38 has a chamber defined by cylindrical portion 40 and conical portion 42. The chamber is closed by a movable wall 44. Specimen 48 is a cylinder having a length greater than the length of the cylindrical portion 40 and having one flat end and a tapered end. The diameter of the cylindrical specimen 48 is substantially less than the diameter of cylindrical portion 40. After compression, there is formed specimen 48' having a cylindrical portion 50 and a tapered portion 52. The tapered portion 52 conforms to the shape of the tapered portion 42 of the chamber while the cylindrical portion 50 conforms to the shape of the cylindrical portion 40 of the chamber. The hardness along cylindrical portion 50 of specimen 48' was as follows. After compression, on specimen 48' the hardness of zone AB did not change, hardness increased from B to C, and was maximum from C to D.

20 In FIG. 9, there is shown a similar press 26 having movable walls 28 and 29 defining a confined cylindrical chamber 30. The specimen 36 has a cylindrical portion 33 and a tapered portion 35. After compression, the specimen 36' had R<sub>A</sub> hardness values as indicated in FIG. 10 at A 69.5, at B 70, and at C 72. At the zone AB the tensile strength was 165,000 psi with 10% elongation and at C the tensile strength was 200,000 psi with 2% elongation.

25 FIG. 12 is a graph of elongation versus percent change of cross sectional area wherein the final size of the specimen was 0.364 inches in diameter and 4.50 inches long. FIG. 13 illustrates a relationship between ultimate tensile strength and percent change in cross-sectional area area for the last mentioned specimen. FIG. 14 is a graph of hardness versus percent change in cross-sectional area for the last mentioned specimen. FIGS. 12-14 relate to an alloy specimen containing 91% tungsten.

30 Test results have shown that there is no difference if only one or both of the walls at opposite ends of the chamber move. The rate of forming was not a significant factor. Substantially identical results were attained when the specimen was offset with respect to the axis of the chamber as opposed to being disposed along the axis of the chamber. In all cases, the hardness increased in proportion to cold work as shown in FIG. 14.

35 The present invention facilitates variation in the strength or hardness in a predetermined manner at a predetermined location along the length of the specimen. No special tooling is required for practicing the present invention. Thus, the invention may be practiced 40 on a conventional hydraulic or mechanical press. The present invention can more efficiently and economically perform functions which were attained heretofore by swaging or forging while achieving features which

cannot be attained by those methods such as excellent surface finish, minimum scrap end losses, closely controlled diameter and length, producing bars with controlled variable mechanical properties.

The procedure for production of a simple cylinder such as specimen 18' is as follows. Determine the desired compressed diameter and length as defined by diameter  $D_2$  and length  $L_2$ . On the basis of the strength required, determine the necessary change in area, for example from the graph of FIG. 13, then select diameter  $D_1$  as required. Calculate initial length  $L_1$  from the constant volume formula:

$$L_1 = \frac{L_2(D_2)^2}{(D_1)^2}$$

Fabricate the specimen to dimensions  $D_1$  and  $L_1$ . Then compress the specimen in a closed chamber as described above.

Thus, the present invention facilitates custom designing by cold working of metals to a pre-determined strength. The rate of movement of the movable wall 16 may vary as desired depending upon the strength of the materials involved. Typical speed of movement of wall 16 is in the range of 0.05 to 200 feet per minute. The metal for the aforesaid specimens may be a tungsten alloy or composite, uranium, steel, or other high strength alloy.

The preformed metal specimens may be made by consolidating powder containing tungsten by a process known generally as sintering. Sintering of powder includes consolidating powdered metal by a number of variations including hot sintering, sintering with pressure and known as hot pressing, sintering without pressure, and hot isostatic pressing.

With respect to a composite, the percentage of copper may vary over a wide range such as 5 to 50%. Favorable results were attained using 70% tungsten and 30% copper powders processed a set forth above.

In FIGS. 15 and 16 there is illustrated one example of a kinetic energy penetrator 60 made from one or more of the final specimens attained in accordance with the method described above. The penetrator 60 when made in accordance with the above description and using the above mentioned tungsten alloy may be used as an anti-tank weapon or other military penetrator type weapon. The method disclosed here permits manufacture of a penetrator having the following features: front and rear ends very hard with the central portion being less hard and having higher elongation; front end very hard with softer central portion and very soft rear end.

The penetrator 60 may have a hard pointed nose 62. When used with a smooth bore weapon, the penetrator may have a stabilizer and sabot. A stabilizing tail cone 64 made from a metal such as aluminum is attached to the end of the projectile remote from nose 62. A sabot 66 engages the ribbed area 68 on the central portion of the penetrator 60. The sabot 66 is preferably made from two or more sections and has cylindrical areas 67 for contact with a smooth bore of a weapon 70. When the projectile 60 is fired from weapon 70, the sabot 66 transfers the force of the propelling gases to the penetrator and thereafter separates into the components thereof as shown in FIG. 14.

The penetrator 60 may have an explosive shaped charge therein with an appropriate delay so that the explosion occurs after penetration by nose 62. The weapon 70 may be stationary or mounted on a vehicle

such as a tank or an airplane. In place of a stabilizing tail cone, stabilizing fins may be utilized.

The present invention can be embodied in other specific forms without departing from the spirit or essential attributes thereof and, accordingly, reference should be made to the appended claims, rather than to the foregoing specification, as indicating the scope of the invention.

I claim:

1. A kinetic energy penetrator comprising a body having a length at least five times as large as its diameter, said penetrator being cold worked so as to have a strength along its length in a predetermined manner attained by the following method:
  - (a) producing a metal specimen with a pre-shape and dimension determined on the basis of the desired strength and mechanical properties,
  - (b) introducing said preshaped specimen into a confined chamber which defines the desired peripheral final shape, spacing at least a portion of the periphery of said preshaped specimen from at least a portion of the walls defining said chamber with the relative dimensions of the spacing being governed by the amount of cold work needed to achieve desired strength or mechanical properties in that portion of the specimen,
  - (c) engaging one face of said specimen with at least one moveable wall of said chamber and applying a continuous compressive force by said wall with a sufficient magnitude to force the preshaped specimen to deform and fill the chamber at the end of the compressive stroke, and
  - (d) applying said compressive force by moving said moveable wall of the chamber so that the yield strength of the specimen progressively increases, and progressively increasing the magnitude of said force as the yield strength increases until the entire circumference of the specimen contacts the walls.
2. The penetrator in accordance with claim 1 wherein step (c) and (d) include deforming the specimen so that all transverse dimensions increased by the same percentage during compression.
3. The penetrator in accordance with claim 1 wherein steps (c) and (d) include deforming the specimen so that transverse dimensions increase by different percentages during compression.
4. The penetrator in accordance with claim 1 wherein steps (c) and (d) are performed with the speed of the moveable wall being sufficiently slow as to cause the specimen to exhibit squirming instability as it increases in transverse dimensions.
5. The penetrator in accordance with claim 1 wherein step (a) includes consolidating powder to produce a metal specimen containing tungsten.
6. The penetrator in accordance with claim 5 wherein step (a) includes sintering powders of tungsten, nickel, iron and cobalt.
7. The penetrator in accordance with claim 1 wherein said penetrator has a pointed nose at one end and stabilizing means at its other end.
8. The penetrator in accordance with claim 1 wherein the hardness of the penetrator adjacent the stabilizing means is substantially the original hardness of the pre-shaped specimen attained by step (a).
9. The penetrator in accordance with claim 8 wherein said penetrator is made from an alloy of tungsten.

10. The penetrator in accordance with claim 1 wherein step (a) includes producing a specimen from uranium, steel, or other high strength alloys.

11. The penetrator in accordance with claim 1 wherein the pre-shaped specimen has a length substantially greater than its transverse dimensions, wherein said movable wall is moved at a speed which is sufficiently slow so as to cause the specimen to exhibit squirming instability as it increases in transverse dimensions, and wherein step (a) is performed in a manner so that 10

steps (c) and (d) produce an article whose hardness varies along its length in a predetermined range.

12. The penetrator in accordance with claim 11 wherein the steps (c) and (d) are applied in a manner so as to cause buckling of the pre-shaped specimen and produce an article at the end of the compressive stroke which has a predetermined hardness at a predetermined location.

\* \* \* \* \*

15

20

25

30

35

40

45

50

55

60

65